

May 15, 1923.

F. J. GROTE, JR

1,455,200

INSULATING COMPOSITION FOR ELECTRICAL APPARATUS

Original Filed Feb. 26, 1920

Fig. 1.



Fig. 2.



Fig. 3.



Inventor

F. J. Grotens, Jr.  
By his Attorneys  
H. C. Tamm.

Patented May 15, 1923.

1,455,200

# UNITED STATES PATENT OFFICE.

FRANK J. GROTE, JR., OF MERIDEN, CONNECTICUT, ASSIGNOR TO THE CONNECTICUT TELEPHONE & ELECTRIC CO., INC., OF MERIDEN, CONNECTICUT, A CORPORATION OF CONNECTICUT.

## INSULATING COMPOSITION FOR ELECTRICAL APPARATUS.

Original application filed February 26, 1920, Serial No. 361,392. Divided and this application filed November 12, 1920. Serial No. 423,649.

To all whom it may concern:

Be it known that I, FRANK J. GROTE, Jr., a citizen of the United States of America, residing at Meriden, New Haven County, 5 Connecticut, have invented a new and useful Insulating Composition for Electrical Apparatus, of which the following is a specification.

The main object of my invention is a compact, durable and efficient construction of coils and condensers for motor ignition work. The adjustments of the ignition system are of course dependent upon the characteristics of the coil and condenser. It is therefore important that all the devices of a given style shall be uniform in every particular so that they will be interchangeable. They must also be capable of quantity production at reasonable cost in order to be 10 available for general use. These devices are subjected to varying electrical conditions and to rough usage. As it is practically impossible for the ordinary user or mechanic to inspect or repair such a device, 15 it should not be subject to deterioration.

To accomplish the best results at a minimum expense, the coils and condensers are first made up according to suitable specifications. The primary coil may consist of 20 one or more layers of suitably insulated wire such as enameled copper. One layer may be wound on a paper tube or on a core and if there is more than one layer, a sheet of insulation such as paper may be interposed 25 between the layers. The secondary may be made up in the same way usually having a large number of layers of smaller wire. The condenser will usually consist of alternate layers of metal foil and fabric, for instance, two strips of foil wound with paper 30 between.

The primary, secondary and condenser elements are then heated for say 40 minutes at about 60° C. They are then preferably 35 dried in a vacuum so that the moisture is sure to be removed without excessive heating. I have found a temperature of 60° C. and a vacuum of about 29 inches of mercury for 40 minutes satisfactory.

The elements are then suddenly immersed 50 in or flooded with a special hot thin liquid compound and subjected to fluid pressure until thoroughly impregnated. This may

take say 30 minutes at a pressure of say 25 to 50 lbs. per square inch, and a temperature of say 130° to 135° C. The compound which I have found gives the best results consists of approximately 85% by weight of a synthetic resin and 15% of oil. The resin I prefer to use is known as "cumar" 55 and consists, I believe, of polymers of paracumarone, para indene and polymers of certain other hydrocarbons obtained from certain coal tar distillates such as crude naphthalene. The polymerization I understand is carried out by the use of sulfuric acid which after the reaction is completed 60 is neutralized with an alkali and the product washed with water and distilled. The melting point depends upon the treatment. 65 This substance has the peculiarity that unlike most gums it can be heated considerably 70 above its melting point without frothing and decomposition. Also it is uniform in quality, free from foreign matter and 75 neither acid or alkali. I prefer to use a product having a melting point of about 80° to 100° C. The oil is preferably China wood oil. The mixture must be very liquid 80 well below the charring temperature of the paper or other spacing material employed so as to completely and uniformly impregnate the element without damage to the insulation. The melting point of the mixture 85 is about 60° C. The resin and oil are heated 90 to a temperature of about 130° C. and mixed so as to be very thin and flow readily when hot. I have found that this compound when handled as above indicated ensures a device with exceedingly high and 95 uniform dielectric properties which is permanent and reliable in character. The coils and condenser for a single device may be assembled before impregnation. This facilitates handling and ensures uniform treatment.

After treatment as above described, the three elements are allowed to drain off excess liquid and then with the usual magnetic core and with a magnetic shield if desired, 100 are surrounded by a casing and a filler compound is poured into the casing and between the elements to more perfectly insulate the parts and keep out all moisture. This filler is preferably composed of the same ingredients as the impregnating compound 105

only I use a resin having a higher melting point, for instance about 130° to 150° C. 84% of this mixed with 16% drying oil and poured at about 180° C. permanently fixes 5 the parts in their proper relation and in no manner affects the impregnating compound and at the same time has the property of regelation at the normal working temperature of the coil so that no damage is done 10 if it is cracked. It will so to speak be "self-healing." The softening point of the filler is about 82° C.

Fig. 1 shows one form of device ready to 15 be impregnated according to my invention (full size).

Fig. 2 shows the same elements as Fig. 1, but located in a casing and filled.

Fig. 3 is a diagrammatic view of apparatus for impregnating according to my invention. 20

It will be understood that I have shown but one form of device, and do not consider my invention as limited to any particular form of coil or condenser, or to any particular combination of coils and condenser. 25

In the particular form shown, 5, 6 and 7 respectively are the primary coil, secondary coil and condenser. The primary coil is shown as wound on a tube 8, a secondary 30 coil on a tube 9 and the condenser has an insulating inner layer 10. The core 11 may be of any suitable type and a magnetic shield 12 may be interposed between the secondary coil and the condenser. The three 35 elements are mounted on a base plate 13 and held together by a rod 14 and cross piece 15. The layer of insulating material 16 is shown interposed between the bottom of the shield, the core and the base plate. 40 Another layer of insulation 17 is shown interposed between the primary and secondary coils and the bottom of the shield 12. As above indicated, the coils and condenser are preferably assembled and impregnated 45 as a unit. After the elements have been impregnated with the compound as above mentioned, a casing such as 18 is placed around the condenser and the filler compound 19 poured in as before referred to.

The impregnating process may be conveniently carried out in apparatus indicated diagrammatically in Fig. 3, where 20 indicates a vat or tank adapted to hold a number of the units to be impregnated, and 21 55 indicates a tank for containing the impregnating compound or mixture of resin and oil. These two tanks may be heated in any suitable way as for instance by steam jackets. The inner chambers of the tanks 60 are connected by a pipe 22 having a valve 23. A pump 24 is connected to the inner chamber of tank 20. A condenser may be used between the pump and the tank. In carrying out the process the elements to be 65 treated are placed in the tank 20 and heated

for say 40 minutes at a temperature of say 60° C. The pump is then started and operated so as to produce a vacuum in the tank 20 of say 29 inches, which is maintained say for an hour and a half. Meanwhile the impregnating compound in the tank 21 is heated to say 130° to 135° C. There is practically no volatilization of the compound under these conditions. At the end of the vacuum drying period the valve 23 is opened 70 and the impregnating liquid sucked over into the tank 20. The valve 23 is then closed and the pump operated until a pressure of say 50 lbs. per square inch is obtained. The coils are left in the impregnating liquid under this pressure for about a half hour and the temperature of the liquid maintained at approximately 130° to 135° C. The valve 23 is then opened and the impregnating liquid which has not been absorbed is forced back into the melting tank 21. The impregnating tank 20 is then 80 opened and the coils allowed to drain for a few minutes. After this, reheating to a temperature above boiling water, say 120° C., will not cause the compound to run out. The coils are then taken out and placed in the casings and filled with the filler compound. As the impregnating compound 85 has a small co-efficient of expansion the element can be taken immediately from the impregnating liquid without danger of cracking, and without causing the layers to separate as the article cools.

I have found that a very high and constant dielectric strength is provided by the use of China wood oil with the "cumar," and that such a compound ensures a most uniform condition and operation of the ignition element. A drying oil such as boiled 100 linseed oil may be used instead of China wood oil, but it should be entirely free of water in order to produce satisfactory results.

It should be understood that I have given the details of only one particular product and the particular steps of the preferred process merely as examples and without intending to limit my claims to the exact proportions, times, temperatures, and pressures given. My invention in the broader aspect 105 covers the treatment of coils or condensers alone or combined.

This process of impregnation not only supplements the insulation on the wire and between the layers of the condenser, but seals it uniformly throughout in case the insulation happens to be defective. The 110 filler compound further protects the coils and condenser, and prevents the absorption 115 of moisture from the air and keeps out surface water, either of which would seriously interfere with the operation of the device if it did not actually ruin it.

The process is claimed in my application 120

#361,392, filed February 26, 1920, from which this is a division.

I claim:

1. An impregnating composition having a melting point of approximately 60° C. comprising a synthetic resin formed from the neutral polymers of para-coumarone, para-indene and other hydrocarbons obtained from a coal tar distillate and mixed with an oil.

2. An impregnating composition comprising approximately 85% of "cumar" and approximately 15% of a drying oil.

3. An impregnating composition of the character described comprising a synthetic resin formed by polymerization of a coal tar distillate and an oil and having a low melting point and a viscosity of from 1½ to 2½ min. by the Engler viscosometer at approximately 130° C.

4. An impregnating composition of the character described having a melting point below 70° C. and composed of from 80% to 93% of a neutral resinous polymerization

product of the cumar and indene group having a melting point of from 70° to 100° C. and from 20% to 7% of oil.

5. An impregnating composition of the character described with a melting point of approximately 60° C. and containing more than 75% of a neutral resinous polymerization product of the cumar and indene group and a drying oil.

6. An impregnating composition of the character described having a melting point of approximately 60° C. and consisting of a major proportion of the neutral polymers of para-coumarone, para-indene and other hydrocarbons obtained from a coal tar distillate and a minor proportion of oil which is miscible with it at a temperature of approximately 130° C. without substantial change.

7. An impregnating composition having a melting point below 100° C. and composed of a major proportion of "cumar" and a minor proportion of oil.

FRANK J. GROTON, JR.